

April 13, 1937.

C. F. LAUENSTEIN

2,077,116

FERROUS ALLOY AND PROCESS OF PRODUCING FERROUS ALLOY

Original Filed April 7, 1933

Fig. 1.



Fig. 2.



Inventor  
Carl F. Lauenstein  
by Parker & Carter.  
Attorneys.

## UNITED STATES PATENT OFFICE

2,077,116

## FERROUS ALLOY AND PROCESS OF PRODUCING FERROUS ALLOY

Carl F. Lauenstein, Indianapolis, Ind., assignor to  
Link-Belt Company, Chicago, Ill., a corporation  
of Illinois

Original application April 7, 1933, Serial No.  
664,902. Divided and this application December  
13, 1934, Serial No. 757,289

6 Claims. (Cl. 148—21.8)

This application is a division of my co-pending application Serial Number 664,902, filed April 7, 1933, which is itself a continuation in part of my application Serial Number 475,829, filed August 5, 1930.

This invention relates to a ferrous alloy and to the process of producing it. The raw material from which the metal is produced is essentially malleableized cast iron which contains certain 10 strengthening alloying elements. Many alloying materials may be used. In the present case I am concerned primarily with the use of manganese, molybdenum, chromium and vanadium which, when alloyed with the iron, form carbides, and 15 may, therefore, be included in "the carbide forming group of alloys". I have also used, however, nickel, copper and aluminum.

As generally understood, ordinary malleableized cast iron is granular in its structure, being composed mainly of grains of ferrite and small particles of carbon or graphitic carbon. One step in the present method or process is designed to cause a combination of the carbon and the ferrite in order to form pearlite or iron carbide.

25 Another object is to produce a metal and a process for making it in which the metal is stronger than ordinary malleableized cast iron and stronger than ordinary malleableized cast iron after it has been treated by my heating 30 process. The presence of the alloying elements in the metal improves the physical properties, particularly improving the ultimate strength, the yield point and the elongation.

Other objects will appear from time to time in 35 the specification and claims.

The metal of the present invention is formed from white cast iron. Before the commencement of my process the iron is put through any standard or suitable malleableizing process. White 40 cast iron has an average chemical composition as follows:

|                  | Per cent  |
|------------------|-----------|
| Combined carbon  | 2.30—2.40 |
| Graphitic carbon | Nil       |
| 45 Silicon       | .90—.95   |
| Manganese        | .27       |
| Sulphur          | .060      |
| Phosphorous      | .16       |

50 To this may be added suitable quantities of copper, molybdenum, nickel, manganese, chromium, vanadium, aluminum or other alloying elements. These alloying elements may be added into the cast iron in the furnace or the ladle, or 55 at any time before the iron is finally molded.

The white cast iron with the alloying elements is poured into suitable molds and allowed to cool. It may then be cleaned and after cleaning it is put through any suitable malleableizing process.

After the malleableizing process is completed 5 a subsequent heat treatment is applied to the metal. This heating will usually be done in furnaces, but may, of course, be done by any other means. The iron is raised to a temperature between 1375° F. and 1500° F. This temperature is 10 given as approximating the best temperature, but a variation either above or below this temperature is possible. After the material has reached the critical or carbon combining temperature a 15 part of the carbon is combined with ferrite. The length of time that the material being treated must be held at this temperature varies with the size of the parts being treated and with the physical properties desired. After the heating 20 has been carried on a sufficient time, the parts are then quenched, that is to say, cooled, in air, oil, water or other medium. In ordinary practice, no particular effort is made to cool the metal slowly and where it is quenched in oil or a liquid, it is usually cooled rapidly. Where it is desired to 25 give the metal a tough and wear resisting outer coat, the heating operation will be carried out in the presence of a carburizing agent.

When the material being treated has been first 30 heated and quenched, it is thereafter reheated to a temperature not exceeding the critical or carbon combining temperature. The result of this second heating is to cause the martensite or troostite retained after the first heating to break down into pearlite or sorbite. This change will 35 normally be effected at a temperature range of 900° F. to 1350° F. The cooling, after the second heating, is preferably air cooling although a water or oil quenching may be used, depending somewhat upon the physical properties desired. A 40 water quenching produces a stiffer, higher strength iron, while oil and air cooling produces relatively more ductile iron. Any cooling method may be used.

The accompanying drawing illustrates in Figure 45 1 the structural arrangement and constituents of a sample of malleableized cast iron and in Figure 2 a sample of the metal of my invention. The figures are diagrammatic showings based upon microphotographs of samples of metals. They 50 suggest diagrammatically only typical forms of the metal. Other samples would show the same general characteristics, but would show detailed modifications.

In Figure 1 the metal is seen to be generally 55

granular. It is composed of grains A, which are ferrite and separated from each other along boundaries B. The grains may be of irregular shapes and sizes. Interspersed through the mass 5 of the metal are spots of free or graphitic carbon C.

Figure 2 is a diagram based upon a microphotograph of a section of a sample of the metal of this invention.

10 As illustrated in the drawing, the metal is generally granular, being formed of grains A. These grains are bounded or separated along boundaries B. The grains are in the form of ferrite. C represents a spot of graphitic or free carbon. In a 15 larger area of the metal, a number of such spots of graphitic carbon would appear. Situated throughout the metal, surrounding the grains and the graphitic carbon and filling the great majority of the grain boundaries and to some degree 20 penetrating within the ferrite grains themselves is pearlite. This material is indicated at D.

Figure 2 illustrates an important characteristic of the present invention, namely, that there is distributed throughout the metal, along the 25 grain boundaries and about such particles of graphitic carbon as are present, an agent which tends to stiffen the grains and prevent their distortion under stress, thus strengthening the mass and preventing the separation or pulling apart of 30 the grains. This agent is an iron carbide with alloy content and in the form illustrated in Figure 2, is normally pearlite or sorbite. It is characteristic of this iron carbide, which in this case may be pearlite or sorbite, that it is strong and 35 tough and it thus strengthens the grains against distortion, holding the grains together more strongly than in other cast iron where the ferrite is combined without the presence of any appreciable amounts of alloy pearlite at the grain 40 boundaries. It thus increases the tensile properties of the material.

It also makes the metal of the invention highly 45 resistant to wear or abrasion. The harder and tougher alloy pearlite or alloy sorbite at the ferrite grain boundaries acts as a guard preventing the wearing or abrading away of the softer ferrite grains. The pearlite or sorbite is strengthened by the alloying element.

In the metal of this invention, the main body 50 of the metal is made up of a group of ferrite grains. The great majority of these grains is surrounded each with a harder shell of pearlite or sorbite, that is to say, with a shell of an iron carbide with alloy content which has such physical 55 properties that it tends to strengthen the grains of ferrite. It prevents deformation of the grain and by this fact it resists distortion of the grain and resists breaking of the grain itself or separation of one grain from the other. This 60 iron carbide in the body of the metal may be said to act like an iron reinforcement about a piece of wood. It prevents distortion and so prevents splitting and breaking. Thus in the metal of this invention there is built up throughout the body 65 of the metal a reinforcing framework of the stronger iron carbide which has many cell-like compartments in it. These cells surround the weaker grains of the ferrite which are thus strengthened and the separation of these ferrite 70 grains is resisted by this cell like structure of the carbide. In effect there is built up a structure which may be likened to a honey comb. This is formed of the iron carbide and within the cells of the honey comb are found the grains of ferrite. 75 The honey comb thus serves to strengthen the

individual grains and to resist deformation of them and further, to resist deformation of the mass as a whole and to prevent separation of the grains.

As above indicated, the metal owes its strength 5 to the presence of the pearlite or some form of iron carbon alloy network surrounding the grains and lying within and along the grain boundaries. The presence of the alloying metal gives this network a higher strength and hardness than 10 that which it would otherwise have if the alloying element were not present.

The temperature ranges above suggested are not absolute limits and are indicated for the first 15 heating as being within the range of the critical or carbon combining temperature, and for the second heating as being above the range of customary hot galvanizing. In the first heating the temperature may be as high as 1500° F. and in the second heating it may be as low as 900° F., 20 although in normal practice the first heating is preferably between 1425° F. and 1450° F. and the second heating is preferably between 1200° F. and 1250° F.

The increased strength of my metal resultant 25 from the use of the alloying element is possibly caused by the pearlite or sorbite, including such an alloy content, having higher physical properties than pearlite or sorbite without this alloy content. This higher strength pearlite or sorbite formed at the grain boundaries has a greater 30 stiffening effect on the ferrite grains and better resists their deformation under stress, thus producing a higher strength metal. Since the physical properties of this alloy pearlite or sorbite, 35 net work can be varied by different heat treatments and by the use of different alloys or different combinations of alloys, the resultant properties of my metal can also be so varied.

The alloying materials above mentioned are 40 only given as typical metals for this use. Many others might be used. For some purposes one will be used along and for other purposes two or more will be used together. Thus one alloy might include manganese, .50 per cent. Another alloy 45 might include molybdenum up to .50 per cent or vanadium up to .60 per cent. These are given as merely typical of possible alloys. One or more of the alloying substances of the carbide forming group may be used in the metal. Thus a very 50 wide variety of alloying elements and combinations of these elements may be used in my invention.

In general, the typical alloying elements and the quantities of them which are most likely to 55 be used are as follows:

|            | Percent     |
|------------|-------------|
| Manganese  | .50 to 1.00 |
| Molybdenum | .20 to .60  |
| Chromium   | .10 to .60  |
| Vanadium   | .10 to .60  |

Where in the claims I have used the expression "a metal of the carbide forming group", consisting of manganese, molybdenum, chromium and vanadium, I mean any one or more of the elements above listed, that is to say, manganese, molybdenum, chromium and vanadium, used generally within the limits above set out. These 65 alloys may be used singly, generally within the 70 ranges indicated, or in any combination of two or more of them.

When the alloying metals are used the annealing or malleableizing cycle is generally the same as that typical of the manufacture of malle- 75

able iron. In some cases the alloy content may necessitate slight variations from the standard. One typical annealing cycle may be as follows: Heat the metal to 1650° F., this heating occupying about 36 hours; hold the metal at 1650° F. for 36 hours. Cool to 1200° F. at 6° F. per hour, occupying about 72 hours. The furnace may then be unloaded and after cooling and inspection the castings or other metal articles may be put 10 through the secondary heat treating cycle. Changes in temperatures and times of heating may be desirable or may be necessary where alloying metals are used or where they are used in different proportions. Some of the elements 15 listed do not have such a marked effect on the critical temperature but in general tend to raise it slightly.

It is therefore possible to use an alloy which depresses the critical temperature, and add to it 20 an alloy which has a slightly opposite or cancelling effect, and use a first treating temperature of 1450° F. In any event, the treating temperatures must be governed by the alloying elements and the desired physical properties in the finished 25 part.

When used alone, manganese tends to lower the critical temperature and an initial heating temperature of 1425° F. to 1475° F. would normally be used, while a second heating of 1200° F. 30 to 1250° F. would normally be used. When molybdenum is used alone, the initial heating temperature is normally in the neighborhood of 1475° F. and the second heating temperature in the neighborhood of 1200° F. A suitable analysis 35 of an alloy involving two of the carbide forming group is as follows:

|             | Percent      |
|-------------|--------------|
| Carbon      | 2.30 to 2.40 |
| Silicon     | .90 to .95   |
| Manganese   | .27          |
| Sulphur     | .06          |
| Phosphorous | .16          |
| Molybdenum  | .30          |

45 Such an alloy would preferably be heat treated by heating to approximately 1500° F., quenching in oil and subsequently reheating to a temperature of 1200° F. to 1250° F.

It is to be understood that a metal with any 50 combination of the various alloying materials is within the contemplation of my invention and thus I might combine manganese, molybdenum, chromium and vanadium all in one metal or any two or any three of them might be combined in 55 one metal.

I claim:

1. A granular ferrous metal, including an alloying element of the carbide forming group of elements consisting of manganese, molybdenum, chromium and vanadium in approximately the following proportions: Manganese .50 to 1.0 per cent; molybdenum .20 to .60 per cent; chromium .10 to .60 per cent and vanadium .10 to .60 per cent, and including ferrite, graphitic carbon and iron carbide, the latter being distributed along 10 the grain boundaries and between the grains of ferrite and about the graphitic carbon.

2. A granular ferrous metal, including at least one of the alloying elements of the carbide-forming group of elements consisting of manganese, 15 molybdenum, chromium and vanadium in approximately the following proportions: Manganese .50 to 1.0 per cent; molybdenum .20 to .60 per cent; chromium .10 to .60 per cent and vanadium .10 to .60 per cent, and including grains of 20 ferrite, graphitic carbon and iron carbide, the latter being distributed along the grain boundaries and between the grains of ferrite and about the graphitic carbon.

3. A granular ferrous metal having an alloying element and including grains of free ferrite, graphitic carbon and iron carbide, the latter being distributed along the grain boundaries and between the grains of ferrite and about the graphitic carbon, said alloying element being 25 molybdenum, from .20 per cent to .60 per cent.

4. A granular ferrous metal having an alloying element and including grains of free ferrite, graphitic carbon and iron carbide, the latter being distributed along the grain boundaries and between the grains of ferrite and about the graphitic carbon, said alloying element being 30 manganese, from .50 per cent to 1.00 per cent.

5. A granular ferrous metal having an alloying element and including grains of free ferrite, graphitic carbon and iron carbide, the latter being distributed along the grain boundaries and between the grains of ferrite and about the graphitic carbon, said alloying element being 35 chromium, from .10 per cent to .60 per cent.

6. The process of heat treating malleableized cast iron, which iron includes an alloying element of the carbide forming group of elements consisting of manganese .50 to 1.0 per cent; molybdenum .20 to .60 per cent; chromium .10 to .60 per cent and vanadium .10 to .60 per cent, which process includes heating the iron to a point between 1375° F. and 1500° F., quenching and reheating to a point between 900° F. and 1350° F.

CARL F. LAUENSTEIN. 55